

Jan. 18, 1927.

1,614,863

D. T. BEATTY

CENTRIFUGALLY CAST PIPE

Original Filed Dec. 2, 1925



INVENTOR

DOUGLAS T. BEATTY

BY  
*J. Granville Meyer*  
ATTORNEY

## UNITED STATES PATENT OFFICE.

DOUGLAS T. BEATTY, OF BIRMINGHAM, ALABAMA, ASSIGNOR TO SAND SPUN PATENTS CORPORATION, OF WILMINGTON, DELAWARE, A CORPORATION OF DELAWARE.

## CENTRIFUGALLY-CAST PIPE.

Original application filed December 2, 1925, Serial No. 30,609. Divided and this application filed June 10, 1926. Serial No. 115,117.

This invention is an improvement in cast hollow bodies, and more particularly in centrifugally cast iron pipes.

mold, but the inclusions are still present, 55 though fairly well disseminated throughout the castings.

These conditions are remedied by centrifugal casting in refractory molds, wherein the lighter impurities are separated by gravity and removed to the inner surface of the casting. The product is further improved by the manner of pouring, wherein the mold is inclined during the pouring, so that the metal enters with practically no rebound or 60 splashing, and in a large, compact body, offering a minimum of surface for cooling and oxidation.

And it is substantially retained in this compact condition until the moment when, 70 by a sudden sharp rise in the speed of rotation of the mold, the molten metal is thrown on to the mold wall, in the second phase of operation, the first phase being that of pouring the molten metal. The mold 75 wall has meanwhile been uniformly heated throughout with fleeting contacts of the large body of metal, so that the third phase of the operation, freezing, takes place under 80 conditions conduced to uniformity of the product.

When hollow bodies are cast in this manner the impurities, such as slag, oxides, sand and the like, of lower specific gravity than the metal tend to deposit on the inner surface of the casting, usually near the ends, in the form of scruff. The union between the layer of scruff and the casting wall may be relatively intimate, thus marring and defacing the surface, and causing pitting of 85 the wall when the scruff layer or coating is removed.

The conditions which result in the formation of scruff may be remedied and the formation of anything approaching an intimate 90 union between the scruff layer and the casting wall may be prevented by careful skimming and surface slagging of the molten metal as it flows on to the mold wall, by the use of a suitable slagging material, such as 95 soda ash. The impurities moved to the inner surface by centrifugal action and the crystallization of the metal, may be converted into a thin, fluid slag with a low fusing point, so that there is a clear separation between the casting wall and the layer of 100 scruff, to facilitate the easy removal of the scruff after setting of the casting.

Hence the conditions which in the previous case caused trouble in the bottom of 105 the mold, are simply transferred to the top of the mold, and no improvement is obtained. In practice a compromise is reached, the iron being poured as hot as possible without serious damage to the top of the

After the metal is poured, within a very short time, from three to six seconds, it is in place on the wall of the mold, and the third phase of the process of casting, which is freezing or crystallization ensues. The freezing begins at the mold and proceeds in one direction only, that is from the outside to the inside. The process may be likened to the growth of trees, premising that their roots are in the mold and their trunks and branches pushing into the freezing metal.

The trunks push into the molten mass, the branches develop and interlock, until the whole cross-section is filled, the trunks proceeding somewhat faster than the branches. This structure, from which originated the expression "dendrites", is visible in steel and white iron, but in gray iron it is obstructed or obliterated by the formation of graphite.

This sequence of crystal formation tends to cleanse the metal by actually pushing the impurities and inclusions out to the inner wall of the pipe, where they are incorporated in the still fluid slag. In prior processes, where the metal cools from both core and mold, the impurities are of necessity trapped between the surfaces. The cleansing action of crystallization is facilitated and aided by centrifugal force acting in the same direction, during the second, casting, and third, freezing, phases. Both forces operate to eliminate slag, gases and sonims.

The betterment of the production obtained by centrifugal casting may be greatly increased by using molds of refractory material, as for instance sand. The sand mold permits slow cooling, which facilitates the operations above mentioned. In addition because of the slow cooling and slow crystallization, the casting is suitable for machining without annealing, which is extremely injurious to the inside gray strata of the pipe, tending as it does to cause the iron to grow. Since the growth is preferential, occurring more rapidly in the gray iron interior than in the white, exterior strains are set up in the outside which tend to weaken this part of the casting.

A uniform distribution of free carbon in the form of graphite is desirable, since "the machinability" of the casting is dependent upon the quantity of residual combined carbon. The deposits of graphite seaming the metal in every direction promote the easy cutting of the tool, since they are weak and also provide lubrication. The deposits of free carbon, that is, graphite, should, however, be of small size, since each flake forms a plane of separation in the sound metal, and the reduction in size and quantity increases the strength of the casting.

One of the primary objects of the present invention is the provision of a centrifugally cast, sand-molded hollow casting, as for in-

stance, a pipe wherein every part of the pipe possesses the same qualities of strength against stresses of every character.

Another object is the provision of a casting of the character specified, substantially free from impurities and from flaws, due to inclusions and the like.

Another object is the provision of a hollow casting of homogeneous structure, wherein the free graphite is in the form of flakes, particles and whorls of relatively small size, but uniformly distributed throughout the structure.

Another object is the provision of a casting wherein the distribution of free carbon in the form of graphite is uniform throughout the structure, with a steady and uniform increase in size of the particles, flakes and whorls through the wall from the exterior to the interior surface.

With these and other objects in view, the invention consists in the improved casting as an article of manufacture.

In the drawings is shown a reproduction of a micro-photograph of the section through the casting wall.

The present case is a division of application No. 30,609, filed December 2nd, 1925.

The casting forming the subject matter of the present invention is produced by spinning or centrifugal casting in a refractory or sand mold. To facilitate charging with a minimum of rebound and splashing, the pouring is done with the mold in inclined position. The charge of molten metal is all, or substantially all, poured while the mold is inclined. During the pouring, the mold is rotated at a relatively low speed, and the sand lining is uniformly heated by fleeting contact with the mass of molten metal, which remains in substantially a compact mass during the operation, offering a minimum surface to oxidation.

During the charging, or near the completion of the charging, the mold is moved quickly but quietly into level position, to uniformly distribute the metal longitudinally of the mold, and at or near the attainment of the mold to level position the speed of rotation is sharply increased, so that the molten metal is thrown upon the mold wall and is held thereon by centrifugal force. Before the metal flows from the ladle it is surface skimmed, and as it flows into the mold, or at any other preferred time, a suitable slagging material, such as soda ash, is added. This material in a finely pulverized condition fuses and blankets the surface of the metal with a thin, extremely fluid slag, and reacting with the silica, carbon dioxide is produced, which drives out the oxygen in the mold, and provides a non-oxidizing atmosphere.

The slagging material, which may be one or more of a number of materials, known as

fluxes, spreads uniformly over the inside surface of the metal, meets the impurities which are moved by gravity into the interior of the casting, and converts them into slag. In addition, the blanket formed by the slag prevents the access of any oxygen which may remain in the pipe to the surface of the metal. The fluxes thoroughly scavenge the metal and the inactive gas evolved prevents reoxidation.

Purification by centrifugal action is furthered by the crystallization which progresses from the exterior toward the interior of the casting, the process of crystallization assisting gravity by pushing impurities to the interior of the casting. The freezing or cooling of the casting progresses radially inward, and a casting is produced wherein the free carbon is in the form of flakes, particles and whorls of relatively small size, but uniformly distributed throughout the structure, as clearly shown in the drawings.

To facilitate comparative consideration of the present casting and those produced in the usual manner in sand molds, the wall may be considered with reference to three zones, namely, those lying adjacent to the outer and inner mold walls, designated A and C, and that between, designated as B. In hollow castings made in sand molds by the usual process, zones A and C are substantially the same, containing primary graphite in a matrix of pearlite with a very little cementite at the extreme edges. Zone B contains primary graphite of much larger size than that in the other zones, in a matrix of pearlite and usually with some free ferrite. The graphite is in the form of flakes and grains of relatively large size. The flakes and grains are of relatively large size, and from the center there is a fairly steady decrease in size toward both surfaces.

In the hollow castings of the present invention, zone A consists in fine primary graphite in a matrix of pearlite, with practically no trace of free cementite, except when extremely hard iron is used. In zone B the graphite is usually in whorls (far superior to flakes) in an almost wholly pearlite matrix. In zone C the flakes of graphite are somewhat larger, being of approximately the same size as those of zone C, in pipes cast by the usual processes. The flakes are in a pearlite matrix, with usually quite a bit of free ferrite.

Zone B of the present pipe occupies normally three-quarters of the total cross section, and the flakes in zone C often run to the very surface of the specimen, a phenomenon which is only possible in castings of the present invention.

When the casting phase commences in

pipes forming the subject matter of the present invention, that is, the laying of the metal on the mold walls, said walls are hot and dry, and the molten metal is in comparatively heavy masses, with no gases trapped by splattering, and covered by a thin, fluid blanket of chemically active slag of lower specific gravity than the iron, much lower freezing point, and fluid through the freezing range of the iron and beyond it.

The improved pipe cast in the manner described, is remarkably free from impurities of every character. There is no chilling of the outer surface such as occurs in casting in metal molds, and the structure of the pipe is uniform throughout, from end to end, and from inner surface to outer surface.

What is claimed as new is:

1. A sand molded pipe, cast centrifugally from skimmed, surface slagged metal in a non-oxidizing atmosphere.

2. A sand molded pipe cast centrifugally from skimmed, surface slagged metal in a non-oxidizing atmosphere, and cooled slowly from the exterior.

3. A pipe composed of iron substantially freed from impurities by skimming, surface slagging and centrifugal casting.

4. A sand molded pipe of metal, surface slagged and centrifugally purified during casting.

5. A sand molded pipe of ferrous metal, surface slagged and centrifugally purified during casting.

6. A sand molded pipe of ferrous metal surface slagged and centrifugally purified in a non-oxidizing atmosphere during casting.

7. An iron pipe of homogeneous metal purified by centrifugal casting and surface slagging, with the free graphite in the form of minute flakes, particles and whorls, extending to the inner face of the casting.

8. An iron pipe of homogeneous metal purified by centrifugal casting and surface slagging, with free graphite in the form of minute flakes, particles and whorls in a matrix of pearlite, uniformly distributed throughout the structure.

9. An iron pipe of homogeneous metal purified by centrifugal casting and surface slagging, with free graphite in the form of minute flakes, particles and whorls in a matrix of pearlite, uniformly distributed throughout the structure, said flakes and particles increasing in size from the exterior to the interior.

Signed at Birmingham, in the county of Jefferson and State of Alabama, this 1st day of June, A. D. 1926.

DOUGLAS T. BEATTY.